

(No Model.)

F. LANNOY.

METHOD OF MAKING FLASHED GLASS.

No. 451,618.

Patented May 5, 1891.

Fig. 1.



Fig. 3.

Fig. 2.



WITNESSES:

*Wm. J. Fether*  
*N. H. Fay*

INVENTOR  
*F. Lannoy*  
BY  
*Charles F. Fay*  
his ATTORNEYS

# UNITED STATES PATENT OFFICE.

FRANCOIS LANNOY, OF TIFFIN, OHIO.

## METHOD OF MAKING FLASHED GLASS.

SPECIFICATION forming part of Letters Patent No. 451,618, dated May 5, 1891.

Application filed December 26, 1890. Serial No. 375,806. (No specimens.)

To all whom it may concern:

Be it known that I, FRANCOIS LANNOY, a citizen of the United States, and a resident of Tiffin, county of Seneca, and State of Ohio, have invented certain new and useful Improvements in Methods of Making Flashed Glass, of which the following is a specification, the principle of the invention being herein explained and the best mode in which I have contemplated applying that principle so as to distinguish it from other inventions.

The object of my invention is to produce variegated "flashed glass"—that is, flashed glass having one of its surfaces composed of two or more colors instead of one solid color, as heretofore.

Heretofore flashed glass has been made as follows: There is gathered on the end of the pontil or blow-tube a small quantity of melted glass or "metal," as it is technically called, of the desired color, and there is then gathered over and around this colored glass a quantity of plain glass sufficient to make a cylinder of the desired size. The combined mass thus formed is then blown in the usual way, and the result is a cylinder composed of two layers, usually of uniform thickness, one layer being formed of plain glass and the other of colored glass of a uniform or solid color. The cylinder is then split longitudinally and flattened in the usual way. By my invention I am enabled to produce a cylinder of glass consisting of two layers, one of which layers shall be formed of plain or other glass, as heretofore described, and the other layer shall be made up of two or more stripes of colored glass of any desired width and color, different shades and colors being as numerous as may be necessary to produce any desired artistic effect.

If the colored layer of the finished sheet of glass is to be made up of, say, six stripes, each of a different color, I would proceed as follows: First. Six pieces of glass of the desired shade of color should be formed of spheroid shape, so that when their edges are placed in contiguity with each other they would fit snugly and compactly together, and the combined pieces would form a figure of substantially bulbous or spheroidal shape, preferably having an open mouth. Second. This spheroidal bulb or cup would then be

placed in a mold or other suitable receptacle that would hold the fitted edges of the different members firmly in contact with each other. The whole should then be slightly heated, so that none of the members would be broken by contact with the highly-heated end of the pontil. Third. A small quantity of melted glass or metal would be gathered around the end of the pontil, the quantity being gaged just sufficient to fit snugly into the open mouth of the bulb, and the pontil thus prepared should be thrust into said mouth or opening. This would cause the sections of the bulb to adhere together and to the end of the pontil. If required, the mass might be slightly blown to cause better and more perfect adhesion to take place. Fourth. Around the bulb so formed is now gathered a quantity of glass sufficient to form a cylinder of the desired size, and the blower proceeds in the usual manner to elongate the entire mass into a cylinder. The prepared sections of the colored glass will thus be caused to form stripes, which may be varied in width and may traverse the cylinder either longitudinally or spirally at the will of the blower, and the artistic effect of the flashed glass thus produced can be varied almost indefinitely by the width of the stripes, the varying shades and colors of the same, and the varied shapes, bends, twists, or curves that the skill of the blower may produce in the stripes.

It should be understood that I by no means limit myself to the spheroid shape of the different members that make up the initial bulb, as any other shape might be used, as desired, provided only that the edges of the different members are so formed as to be capable of adhering to each other and making one common bulb that might afterward be treated and finished by blowing. Neither do I limit myself to placing the combined members in a mold previous to inserting the pontil, as any apparatus or process causing the separate members to adhere to each other would be as effectual.

Referring to the drawings, Figure 1 is a perspective view of a spheroid-shaped piece of glass of any solid color. Fig. 2 is a perspective view of a bulbous or spheroidal shaped figure made up of several of the sec-

toral-shaped figures shown in Fig. 1, having their edges joined; and Fig. 3 is a sectional view of the glass bulb ready for blowing.

The letter A represents one of the spheroidal sectoral pieces or members that go to make up the bulb B, from which a cylinder may be blown.

The foregoing description and accompanying drawings set forth in detail one method of carrying out my invention. Change may be made therein, provided the principles of operation respectively recited in the following claims are employed.

I therefore particularly point out and distinctly claim as my invention—

1. A method of making flashed glass, consisting of joining and causing to adhere the edges of two pieces of glass of different shades, then coating the combined piece thus made with molten glass, and blowing the mass, substantially as set forth.

2. A method of making variegated flashed glass, consisting of uniting the edges of two pieces of glass of different colors so as to form a bulb, inserting the blow-tube in the opening in said bulb, then coating the bulb with glass of a solid color, and then blowing the coated bulb, substantially as set forth.

3. A method of making variegated flashed glass, consisting of joining the edges of two

or more pieces of glass of different colors, the combined pieces substantially of spheroidal form, placing the spheroid in a mold and holding the pieces composing it together and slightly heating them, blowing the spheroid and causing the edges to unite, coating the mass thus formed with plain glass, and blowing the same, substantially as set forth.

4. In a method of making variegated flashed glass, the following steps: first, shaping pieces of glass of different colors of substantially spheroid-sectoral form, so that when their edges are brought into contact they form a bulb with an open mouth, placing the bulb in a mold and slightly heating it, inserting a tube provided with metal in the open mouth of said bulb and blowing sufficiently to attach the metal to the bulb and cause the contiguous edges of the sectoral pieces to adhere, then withdrawing the bulb from the mold, coating it with plain glass, and blowing the combined mass, substantially as set forth.

In testimony that I claim the foregoing to be my invention I have hereunto set my hand this 13th day of December, A. D. 1890.

FRANCOIS LANNOY.

Witnesses:

T. L. MAGERS,  
J. E. MAGERS.